

## UNITED STATES PATENT OFFICE

AUGUST E. SCHUTTE, OF NORTHBORO, MASSACHUSETTS

## METHOD OF WATERPROOFING PILES

No Drawing.

Application filed March 7, 1928. Serial No. 259,930.

My invention refers to concrete piling, or plain, or re-enforced concrete structures, which are waterproofed and rendered stronger and more durable by impregnating the same with asphalt or bituminous material. I am aware that concrete piling has been manufactured by impregnating the surface, or the entire mass, with asphalt, by saturation but all these processes so far as I am aware require the immersion of the pile in the asphalt, either partially or completely. This necessitates the handling and moving of the pile, which is always a costly operation. Under the present method, the pile can be given a superficial coating of asphalt, which penetrates the desired distance into the concrete, and during the operation the pile does not have to be immersed, lifted, or handled.

By my method I treat the pile superficially with an exceedingly hot asphalt of any desired penetration. This is done by applying to one surface of the pile an asphalt which can be applied either hot or cold, and then applying intense heat thereto, the heating being carried to a degree above the flash point of the asphalt. The asphalt is thus liquefied so that it readily enters the pores and at the same time, due to the high temperature employed, the concrete is dried out both by the heating medium and the highly heated asphalt.

The intense heat, as will be seen, serves a double purpose, it evaporates the water in the concrete and heats the latter, and as soon as the pores and voids are cleared of moisture, the intensely heated and therefore very liquid asphalt enters the pores and effectually seals them, leaving a continuous bituminous surface on the outside. It is obvious that the depth of impregnation can be controlled by the length of heating and the amount of asphalt applied. From one-quarter to one-half inch is usually sufficient, but two and three inches can be easily achieved or even complete saturation is possible.

To practice my invention, I form a pile, plain or re-enforced in the usual way and allow it to cure until a desired strength is

secured. I then either paint or sprinkle this surface with asphalt, and apply to such treated surface an intense heat. This can be done, either by a direct flame, by superheated steam, superheated air, hot iron smoothers, or any desired source of heat. As soon as the heat is applied, it will be noticed that the moisture forms steam bubbles in the asphalt surface, and that continued heating allows the steam to escape through the thin very hot film of asphalt which is so liquid that it enters all the small voids and crevices, and saturates and impregnates the concrete structure. This process can be continued until desired penetration is achieved. The outside coating can be thickened, if desired, by another application of asphalt. As soon as the pile is cool it is ready to use.

The action of heat, used as described in my process, is entirely different from the action of heat contained in a body of hot bituminous material applied directly to a concrete surface. If a heated asphalt is applied to a concrete surface, the heat is only of momentary duration, hottest immediately at the application of the hot material, and cooling rapidly. Such heat evaporates the moisture of the concrete and forms bubbles or thin layers of moisture below the asphalt, or rather at the plane of contact of the asphalt and the concrete with no means of escape. Such layer can be peeled off as soon as it is cool for it does not adhere to the concrete on account of that film of moisture. If, however, as in my process, the surface is first coated with an asphalt and intense heat is applied, the asphalt is heated to near or above its flash point, and the concrete below it is heated, causing the moisture to evaporate and escape through the fluid film of asphalt. As soon as the steam escapes, the asphalt enters the pores and penetrates into the structure. This process can be continued by applying more asphalt and more heat until the desired degree of impregnation is obtained.

It is to be understood that the method is not to be limited to a treatment at one and the same time over the entire surface of the piling or structure, but it may be effect-

ed step by step or portion by portion, until the entire surface has been treated.

What is claimed is:

- 5 A method of waterproofing and strengthening concrete pile by first applying heat to the concrete, evaporating the moisture locally and at the surface, applying an asphalt, subjecting said asphalt superficially to an intense heat until it penetrates to the
- 10 desired depth, applying more asphalt and continuing the process until a desired penetration has been achieved, and proceeding thus from spot to spot until the entire surface has been covered.
- 15 In testimony whereof I have signed my name to this specification.

AUGUST E. SCHUTTE.

20

25

30

35

40

45

50

55

60

65